# EUROPEAN PATENT SPECIFICATION

(11) **EP 2 652 189 B1**
(45) Date of publication and mention of the grant of the patent: **14.02.2018**
(21) Application number: 11864804.7
(22) Date of filing: 16.12.2011
(51) Int. Cl.: D04H 1/00

(54) **FINE FIBER FILTER MEDIA AND PROCESSES**
FEINFASER-FILTERMEDIEN UND VERFAHREN DAFÜR
MILIEU FILTRANT À FIBRES FINES ET PROCÉDÉS CORRESPONDANTS

(30) Priority: 17.12.2010 US 971594; 17.12.2010 US 971539
(43) Date of publication of application: 23.10.2013
(73) Proprietor: Hollingsworth & Vose Company, East Walpole, MA 02032 (US)
(72) Inventor: COX, Stephen, T., Radford, VA 24141 (US); FREEMAN, William, S., Roanoke, VA 24018 (US)
(74) Representative: Hoffmann Eitle
(86) International application number: PCT/US2011/065499
(87) International publication number: WO 2012/150964

(56) References cited:
- WO-A1-2010/101640
- WO-A2-2009/062009
- US-A1- 2006 084 341
- US-A1- 2008 026 659
- US-A1- 2008 318 014

## Description

### FIELD

Fine fiber products, including those suitable for use as filter media, as well as related assemblies, systems and methods, are described.

### BACKGROUND

Filter media can be used to remove contamination in a variety of applications. Depending on the application, the filter media may be designed to have different performance characteristics. In general, filter media can be formed of a web of fibers. The fiber web provides a porous structure that permits fluid (e.g., a liquid or a gas) to flow through the filter media. Contaminant particles contained within the fluid may be trapped on the fibrous web. Filter media characteristics, such as fiber diameter and basis weight, affect filter performance including filter efficiency and resistance to fluid flow through the filter.

Fiber webs can be formed by different processes. In a meltblowing process, a fiber web may be formed by extruding a polymeric material through a die and then attenuating the resulting filaments with a heated, high-velocity air stream. This process may generate fine fibers that can be collected onto a moving collector belt where they intertwine with each other to form a fiber web. There are several parameters during the extrusion process that can affect the structural and performance characteristics of the resulting fiber webs. Improvements in the extrusion process may lead to fiber webs having improved structural and performance characteristics, such as reduced fiber diameters, increased surface area, and/or reduced basis weight. Such improvements would find use in a number of different fields where fiber webs can be used, such as in filtration applications.

Document WO 2010/101640 A1 describes filter media that have a layer with a waved configuration in order to increase the surface area, which can be used as filter elements in applications.

In document WO 2009/062009 A2 filter media are obtained by using one or more layers of a meltblown assembly of one or more polymers.

### SUMMARY

The disclosure generally relates to fine fiber products, as well as related assemblies, systems and methods.

In the following, the units "CFM" (cubic feet per minute), "inch", "particles/in²", "lbs/hr", "°F" can be converted into the corresponding SI units by using by the respective conversion factors:
1 CFM = 0.0283 m³/min
1 inch = 25.4 mm
1 particles/in² = 0.155 particles/mm²
1 lbs/hr = 0.454 kg/h
$T \left[K\right] = \left(T \left[° F\right] + 459.67\right) \times 5 / 9.$ In some embodiments, a series of fiber webs are provided. In one set of embodiments of the present disclosure, a fiber web includes a plurality of meltblown fibers formed of a polymeric material and having an average fiber diameter between about 0.1 microns and about 1.5 microns. The fiber web has an air permeability between about 10 CFM and about 1800 CFM, a surface area between about 0.1 m²/g and about 6.0 m²/g, a basis weight between about 1.0 g/m² and about 100 g/m², and a thickness between about 0.0005 inches and about 0.04 inches. The fiber web also has a surface density of particles formed of the polymeric material of less than about 1.6 particles/in², wherein each of the particles has a largest cross-sectional dimension of about 1.0 mm or greater. In another set of embodiments of the present disclosure, a fiber web includes a plurality of meltblown fibers formed of a polymeric material and having an average fiber diameter between about 0.1 microns and about 0.6 microns. The fiber web has an air permeability between about 10 CFM and about 1800 CFM, a surface area between about 0.1 m²/g and about 6.0 m²/g, a basis weight between about 1.0 g/m² and about 100 g/m², and a thickness between about 0.0005 inches and about 0.04 inches. The fiber web also has a surface density of particles formed of the polymeric material of less than about 5 particles/in², wherein each of the particles has a largest cross-sectional dimension of about 1.0 mm or greater.

In one set of embodiments according to the present invention, a fiber web includes a plurality of meltblown fibers having an average fiber diameter between about 0.1 microns and about 1.5 microns. The fiber web has an air permeability between about 10 and about 1800 CFM, a surface area greater than about 2.0 m²/g, a basis weight between about 1.0 g/m² and about 100 g/m², and a thickness between about 0.0005 inches and about 0.04 inches.

In some embodiments of the present disclosure, a series of methods of forming fiber webs is provided. In one set of embodiments of the present disclosure, a method of forming a fiber web includes introducing a polymeric material into an extrusion system including an extruder inlet, a die outlet, and a processing space between the extruder inlet and the die outlet, wherein the extrusion system comprises a extruder barrel having an inner diameter of about 4 inches or less, and processing the polymeric material in the extrusion system such that the polymeric material has a dwell time of less than about 85 minutes in the processing space. The method also includes forming a plurality of meltblown fibers from the polymeric material, wherein the plurality of meltblown fibers have an average diameter between about 0.1 microns and about 1.5 microns, and forming a fiber web comprising the plurality of meltblown fibers.

In another set of embodiments of the present disclosure, a method of forming a fiber web includes introducing a polymeric material into an extrusion system including an extruder inlet, a die outlet, and a processing space between the extruder inlet and the die outlet having a volume of less than about 25,000 cm³. The method also includes forming a plurality of meltblown fibers from the polymeric material, wherein the plurality of meltblown fibers have an average diameter between about 0.1 microns and about 1.5 microns, and forming a fiber web comprising the plurality of meltblown fibers.

In another set of embodiments of the present disclosure, a method of forming a fiber web includes introducing a polymeric material into an extrusion system including an extruder inlet, a die outlet, and a processing space between the extruder inlet and the die outlet, and processing the polymeric material in the extrusion system such that the polymeric material has a dwell time in the processing space of less than about 30 minutes and a throughput of less than about 85 lbs/hr. The method also includes forming a plurality of meltblown fibers from the polymeric material, wherein the plurality of meltblown fibers have an average diameter between about 0.1 microns and about 1.5 microns, and forming a fiber web comprising the plurality of meltblown fibers.

In another set of embodiments of the present disclosure, a method of forming a fiber web includes introducing a polymeric material into an extrusion system including an extruder inlet, a die outlet, and a processing space between the extruder inlet and the die outlet, and processing the polymeric material in the extrusion system such that the polymeric material has a dwell time in the processing space of less than about 50 minutes and a throughput of less than about 55 lbs/hr. The method also includes forming a plurality of meltblown fibers from the polymeric material, wherein the plurality of meltblown fibers have an average diameter between about 0.1 microns and about 1.5 microns, and forming a fiber web comprising the plurality of meltblown fibers.

Other advantages and novel features of the present invention will become apparent from the following detailed description of various non-limiting embodiments of the invention when considered in conjunction with the accompanying figures.

### BRIEF DESCRIPTION OF THE FIGURES

Non-limiting embodiments of the present invention will be described by way of example with reference to the accompanying figure, which is schematic and is not intended to be drawn to scale. In the figure, each identical or nearly identical component illustrated is typically represented by a single numeral. For purposes of clarity, not every component is labeled, nor is every component of each embodiment of the invention shown where illustration is not necessary to allow those of ordinary skill in the art to understand the invention. In the figures:
FIG. 1 is a schematic diagram showing a process for fiber formation according to one set of embodiments of the present disclosure.

### DETAILED DESCRIPTION

Fine fiber products including fiber webs, as well as related assemblies, systems and methods, are described. In some embodiments, fiber webs described herein may include fine fibers and relatively low amounts of degraded polymer formed during a fiber extrusion process. Polymer degradation may result in the formation of polymeric particles, which may lessen the properties of fiber webs used for filter media or other applications. Polymer degradation may be decreased by, for example, decreasing the amount of time (e.g., dwell time) the polymeric material spends at relatively high temperatures and pressures in certain portions of the extrusion system. Factors influencing this decreased dwell time are balanced with the desire to form fibers having small diameters which in certain conventional processes are produced at longer dwell times. In some embodiments, fiber webs described herein have a relatively low air permeability and a relatively high surface area, which can lead to increased performance. Other advantages of the articles, methods and systems described herein are also provided.

This disclosure describes several methods for addressing some problems associated with certain polymer fiber extrusion processes. One problem involves the formation of fibers having very small diameters. As described in more detail below, generally the formation of fibers having very small diameters in certain extrusion processes uses a relatively low polymer throughput. However, a low throughput may lead to the formation of degraded polymeric material in the form of particles during an extrusion process. This degradation may be caused by the polymeric material being subjected to the relatively high temperatures and pressures of the extrusion process for prolonged periods of time and/or to other conditions. As the amount of degraded polymer increases, less fiber is produced per unit of polymer. For fiber webs used for filtration or certain other applications, this occurrence is not desirable as it may result in having to form fiber webs having a higher basis weight in order to achieve the same level of performance as fiber webs without degraded polymer, all other factors being equal.

In the past, increased amounts of degraded polymer formed during an extrusion process sometimes results in the practitioner having to change certain parameters of the extrusion process to reduce the amount of degraded polymer; however, these changes may lead to the formation of fibers having relatively larger diameters and/or fiber webs having less desirable performance characteristics. The inventors have discovered within the context of the invention that by balancing certain parameters of an extrusion process and/or by including one or more additives to the polymeric material used to form the fibers, fine fiber webs having relatively low amounts of polymer degradation, increased performance, and/or better structural characteristics can be achieved. Examples of parameters that can be varied and additives that can be used to achieve this result are described in more detail below.

Although much of the description provided herein refers to a fiber web or a meltblown product used as filter media, it should be understood that the fiber web and/or meltblown product can be used in other applications in other embodiments.

FIG. 1 shows a system 1 that may be used in methods that form fine fibers according to certain embodiments described herein. As shown in this illustrative embodiment, a polymeric material 10, such as a resin which may be in granular form, may be introduced into a mixer 20, where the polymeric material can be optionally combined with one more additives. The polymeric material may then be transported in the direction of arrows 22 towards an inlet 24 of an extruder 25. The extruder includes an extruder screw 26 that is mounted for rotation within an extruder barrel 27. Through the rotation of the screw, polymeric material is conveyed downstream within the extruder barrel, which may be heated to a desired temperature to create a fluid stream of polymeric material. The polymer is heated (generally slowly) from the inlet of the extruder to the outlet of the extruder to allow the polymeric material to flow more easily. The stream of polymeric material may then flow into one or more conduits 28 fluidically connecting the extruder to a die body 30 (e.g., connecting the extruder outlet to a die body inlet). The volume between the extruder inlet and a die outlet 44 collectively define a processing space having a particular internal volume that can be used to calculate the dwell time of the polymeric material, as described in more detail below.

As shown illustratively in FIG. 1, a melt pump 32 may be positioned between conduit 28 and the die body. The melt pump can help control the amount of polymer throughput (lb/hr) delivered to the die body. The die body has a die temperature which influences the temperature of the polymeric material in the die body, including the temperature of the polymer in a spin pack 40 connected to the die body. The spin pack may include one or more channels 42 allowing the polymer to flow towards a die outlet 44 (e.g., a die tip) including one or more holes. The spin pack also includes one or more additional channels 46 which can allow air or other gases to flow towards the die tip. As the melted polymer exits the one or more die outlets, the air flowing in channels 46 attenuates the polymer into fibers. Fiber formation can be controlled by modifying the process air temperature and process air volume.

The polymer exiting the one or more holes of the die outlet is formed into meltblown fibers 50 onto a collector table 60 which includes a collector belt 70. The diameter of the fibers may be controlled in part by air or other gases introduced into channels 55, which can be used to quench the fibers. The heated, high velocity air impinges the polymer on either side of the die outlet as the polymer exits out of the die outlet. This air may attenuate the fiber to the final fiber size. Quenching can be controlled by modifying the quench air temperature and quench air volume.

The fibers collected onto the collector belt may be pulled towards the collector table using a suction box 74. The fibers collected onto the collector belt form a fiber web. The distance 75 from the die tip to the collector table can be varied to control the density of the fiber web (e.g., as the distance is increased, the fiber velocity is decreased and the fiber temperature is reduced so packing of the fibers is less dense, resulting in a more lofty web). As the distance is increased, the velocity of the fiber is generally decreased, making a loftier fiber web. The collector suction is also controlled, which also impacts the loft of the fiber web. The basis weight and thickness of the fiber web can be varied by controlling the collector belt speed. The collector belt transports the fiber web to a winder 80 where the fiber web can be further processed if desired.

In certain embodiments of the present disclosure, a method of forming a fiber web may involve controlling the dwell time of the polymeric material in a processing space of a system such as the one shown in FIG. 1. The dwell time is the time the polymeric material spends in a processing space, which includes the combined volume where the polymeric material can reside between an extruder inlet and a die outlet, within the temperature- and pressure-controlled confines of the extrusion process. The combined volume may include, for example, the volume of the extruder (e.g., extruder barrel), die body, and any conduits fluidically connecting the extruder and die body. The dwell time can be calculated using the formula: $Dwell time = V ⋅ ρ / Th$ where V is the volume of the processing space as defined above, ρ is the density of the polymeric material being extruded, and Th is the throughput of the polymeric material through the die body.

Without wishing to be bound by any theory, the inventors believe that in some embodiments of the present disclosure, in order to form fine fiber webs, relatively low throughputs may be used during the extrusion process. Relatively low throughputs allow fibers having small diameters to be formed; however, low throughputs may also result in a certain amount of the polymeric material used to form the fibers to become degraded due to the polymeric material being subjected to the relatively high temperatures and pressures of the extrusion process for prolonged periods of time (i.e., a relatively high dwell time). Degradation may result in the formation of small polymeric particles as described in more detail below, which may lessen the filtration properties of the fiber web. If relatively high throughputs are used, the dwell time of the polymeric material decreases; however, fibers having larger diameters may be formed. As a result, in some embodiments of the present disclosure, a suitable process for forming fine fibers with low polymer degradation may involve balancing both the throughput and the dwell time of the polymeric material during the extrusion process.

The inventors have recognized within the context of the invention that one method for decreasing the dwell time of the polymeric material while obtaining small fiber diameters is to decrease the volume of the processing space. As the processing space includes the combined volume between an extruder inlet and a die outlet, the volume of the processing space may be decreased by, for example, decreasing the diameter and/or length of the extruder barrel, decreasing the number, diameter and/or length of any conduits connecting the extruder and die body, decreasing the internal volume of the die body, and combinations thereof. Using a relatively low processing space volume during an extrusion process can allow, in some embodiments of the present disclosure, a relatively low polymer throughput to be used, while still maintaining a relatively low dwell time. As such, fine fiber webs having relatively low polymer degradation may be formed.

The inventors have also observed within the context of the invention that in some embodiments of the present disclosure, the temperature of the polymeric material in the processing space may have relatively little effect on the amount of polymer degradation, e.g., compared to the dwell time. One of ordinary skill in the art would have expected that polymer degradation was caused by the polymeric material being subjected to the relatively high temperatures (and pressures) during the extrusion process. Accordingly, to decrease the amount of polymer degradation, one of ordinary skill in the art would likely decrease the temperature of the polymeric material in the extruder and/or die body. One of ordinary skill in the art would not have expected that low amounts of polymer degradation can be achieved while using relatively high processing temperatures in combination with modifying other parameters as described in certain methods provided herein.

As noted above, in some embodiments of the present disclosure, a method of forming a fiber web may involve controlling the dwell time of the polymeric material in a processing space of an extrusion system. In certain embodiments, the dwell time may range between about 1 minute and about 2,600 minutes. For example, the dwell time of the polymeric material may be between about 1 minute and about 1,500 minutes, between about 2 minutes and about 1,000 minutes, between about 2 minutes and about 500 minutes, between about 2 minutes and about 100 minutes, between about 3 minutes and about 90 minutes, between about 5 minutes and about 76 minutes, between about 5 minutes and about 50 minutes, between about 5 minutes and about 30 minutes, or between about 1 minute and about 15 minutes. In some embodiments, the dwell time of a polymeric material in a processing space is less than about 2,000 minutes, less than about 1,500 minutes, less than about 1,000 minutes, less than about 500 minutes, less than about 200 minutes, less than about 100 minutes, less than about 75 minutes, less than about 50 minutes, less than about 30 minutes, less than about 20 minutes, less than about 15 minutes, less than about 10 minutes, or less than about 5 minutes. Other ranges and values of dwell time are also possible.

The polymer throughput may range, for example, between about 1 lb/hour and about 200 lbs/hour. For instance, the polymer throughput may be between about 11b/hour and 150 lbs/hours, between about 11b/hour and 100 lbs/hour, between about 2 lbs/hour and about 90 lbs/hour, between about 20 lbs/hour and about 85 lbs/hour, between about 20 lbs/hour and about 60 lbs/hour, between about 40 lbs/hour and about 85 lbs/hour, or between about 1 lb/hour and 20 lbs/hour. In some embodiments of the present disclosure, the polymer throughput may be less than about 200 lbs/hour, less than about 150 lbs/hour, less than about 100 lbs/hour, less than about 85 lbs/hour, less than about 60 lbs/hour, less than about 40 lbs/hour, less than about 20 lbs/hour. In other embodiments, the polymer throughput may be greater than about 20 lbs/hour, greater than about 40 lbs/hour, greater than about 85 lbs/hour, greater than about 100 lbs/hour, greater than about 150 lbs/hour, or greater than about 200 lbs/hour. Other ranges and values of polymer throughput are also possible.

The volume of the processing space where polymeric material can reside may be varied in some embodiments of the present disclosure, e.g., to achieve a particular dwell time. The volume of the processing space may range, for example, between about 10 cm³ and about 30,000 cm³, between about 10 cm³ and about 25,000 cm³, between about 10 cm³ and about 20,000 cm³, between about 10 cm³ and about 15,000 cm³, between about 10 cm³ and about 12,000 cm³, between about 10 cm³ and about 10,000 cm³, between about 10 cm³ and about 8,000 cm³, between about 10 cm³ and about 6,000 cm³, between about 10 cm³ and about 4,000 cm³, between about 10 cm³ and about 2,000 cm³, between about 10 cm³ and about 1,000 cm³, or between about 10 cm³ and about 500 cm³. In some cases, the volume of the processing space is less than about 30,000 cm³, less than about 25,000 cm³, less than about 20,000 cm³, less than about 15,000 cm³, less than about 12,000 cm³, less than about 10,000 cm³, less than about 8,000 cm³, less than about 6,000 cm³, less than about 4,000 cm³, less than 2,000 cm³, less than about 1,000 cm³, or less than about 500 cm³. Other ranges and values of processing space volume are also possible.

The size of the extruder screw (e.g., screw diameter) may be varied in some embodiments of the present disclosure, e.g., to achieve a particular processing space volume. In some embodiments, the extruder screw diameter may be between about 0.25 and about 6.0 inches. For instance, the extruder screw diameter may be between about 0.25 inches and about 5.5 inches, between about 0.5 inches and about 5.0 inches, between about 1.0 inch and about 4.0 inches, between about 1.0 inch and about 3.5 inches, or between about 1.0 inch and about 3.0 inches. In some cases, extruder screw diameter may be about 6.0 inches or less, about 5.5 inches or less, about 5.0 inches or less, about 4.5 inches or less, about 4.0 inches or less, about 3.5 inches or less, about 3.0 inches or less, about 2.5 inches or less, about 2.0 inches or less, or about 1.5 inches or less. Other ranges and values of extruder screw diameters are also possible.

The extruder barrel diameter (e.g., the inner diameter of the barrel) may be varied in some embodiments of the present disclosure and may be chosen to match the size of the extruder screw. For example, an extruder screw having a 4 inch diameter may be matched with an extruder barrel having an inner diameter of about 4.0 inches. In some embodiments, the extruder barrel may have an inner diameter of between about 0.25 and about 6.0 inches. For instance, the inner diameter of the extruder barrel may be between about 0.25 inches and about 5.5 inches, between about 0.5 inches and about 5.0 inches, between about 1.0 inch and about 4.0 inches, between about 1.0 inch and about 3.5 inches, or between about 1.0 inch and about 3.0 inches. In some cases, the inner diameter of the extruder barrel may be about 6.0 inches or less, about 5.5 inches or less, about 5.0 inches or less, about 4.5 inches or less, about 4.0 inches or less, about 3.5 inches or less, about 3.0 inches or less, about 2.5 inches or less, about 2.0 inches or less, or about 1.5 inches or less. Other ranges and values of extruder barrel inner diameters are also possible.

In certain embodiments of the present disclosure, the length of the extruder barrel may be varied, e.g., to achieve a particular processing space volume. In some embodiments, the length of the extruder barrel may be between about 1 ft and about 15 ft. For instance, the length of the extruder barrel may be between about 1 ft and about 12 ft, between about 1 ft and about 10 ft, between about 1 ft and about 8 ft, between about 1 ft and about 6 ft, between about 1 ft and about 5 ft, between about 1 ft and about 4 ft, or between about 1 ft and about 2 ft. In some cases, the length of the extruder barrel is about 15 ft or less, about 12 ft or less, about 10 ft or less, about 8 ft or less, about 6 ft or less, about 5 ft or less, about 4 ft or less, about 3 ft or less, or about 2 ft or less. Other ranges and values of extruder barrel lengths are also possible.

In certain embodiments of the present disclosure, the average diameter of one or more conduits between an extruder outlet and a die inlet (e.g., space where a polymeric material can reside) may be varied, e.g., to achieve a particular processing space volume. In some embodiments, the average conduit diameter may be between about 0.1 and about 10.0 inches. For instance, the average conduit diameter may be between about 0.3 inches and about 8.0 inches, between about 0.3 inches and about 5.0 inches, between about 0.1 inches and about 3.0 inches, between about 0.1 inches and about 2.0 inches, between about 0.5 inches and about 2.0 inches, between about 0.1 inches and about 1.8 inches, between about 0.1 inches and about 1.6 inches, between about 0.1 inches and about 1.4 inches, between about 0.1 inches and about 1.2 inches, between about 0.1 inches and about 1.0 inches, or between about 0.1 inches and about 0.8 inches. In some cases, the average conduit diameter is about 10.0 inches or less, about 8.0 inches or less, about 6.0 inches or less, about 4.0 inches or less, about 3.0 inches or less, about 2.0 inches or less, about 1.8 inches or less, about 1.6 inches or less, about 1.4 inches or less, about 1.2 inches or less, about 1.0 inches or less, about 0.8 inches or less, or about 0.7 inches or less. Other ranges and values of average conduit diameters are also possible.

In certain embodiments of the present disclosure, the combined length of one or more conduits between an extruder outlet and a die inlet (e.g., space where a polymeric material can reside) may be varied, e.g., to achieve a particular processing space volume. In some embodiments, the combined conduit length may be between about 0.5 ft and about 75 ft. For instance, the combined conduit length may be between about 5 ft and about 50 ft, between about 5 ft and about 40 ft, between about 5 ft and about 30 ft, between about 10 ft and about 25 ft, between about 5 ft and about 25 ft, between about 5 ft and about 20 ft, between about 5 ft and about 15 ft, between about 1 ft and about 12 ft, between about 1 ft and about 10 ft, between about 1 ft and about 8 ft. In some cases, the conduit length may be about 75 ft or less, about 50 ft or less, about 40 ft or less, about 30 ft or less, about 25 ft or less, about 20 ft or less, about 15 ft or less, about 12 ft or less, about 10 ft or less, about 8 ft or less, or about 6 ft or less. Other ranges and values of combined conduit lengths are also possible.

The volume of the die body (including the spin pack) where polymeric material can reside may be varied in some embodiments of the present disclosure. The volume of the die body may range, for example, between about 300 cm³ and about 15,000 cm³, between about 300 cm³ and about 13,000 cm³, between about 300 cm³ and about 11,000 cm³, between about 300 cm³ and about 9,000 cm³, between about 300 cm³ and about 6,000 cm³, between about 300 cm³ and about 4,000 cm³, between about 300 cm³ and about 2,000 cm³, between about 300 cm³ and about 1,000 cm³, or between about 300 cm³ and about 600 cm³. In some cases, the volume of the die body is 15,000 cm³, less than about 13,000 cm³, less than about 10,000 cm³, less than about 8,000 cm³, less than about 6,000 cm³, less than about 4,000 cm³, less than 2,000 cm³, less than about 1,000 cm³, or less than about 600 cm³. Other ranges and values of die volume are also possible.

In some embodiments of the present disclosure, an extrusion process described herein may include a particular die temperature range or value. In general, the die temperature may be selected to suitably soften (e.g., melt) the polymeric material that is to be formed into fibers. In some embodiments, the die temperature is between about 400 °F and about 630 °F. For instance, the die temperature may be between about 410 °F and about 600 °F, between about 410 °F and about 580 °F, between about 420 °F and about 550 °F, between about 420 °F and about 500 °F, or between about 530 °F and about 550 °F. In certain embodiments, the die temperature may be greater than about 400 °F, greater than about 420 °F, greater than about 440 °F, greater than about 460 °F, greater than about 480 °F, or greater than about 500 °F. In other embodiments, the die temperature may be less than about 630 °F, less than about 550 °F, less than about 530 °F, less than about 520 °F, less than about 500 °F, or less than about 450 °F. Other ranges and values of die temperatures are also possible.

The temperature of the extruder barrel typically varies from the inlet of the extruder to the outlet of the extruder to allow the polymeric material to flow more easily. The minimum temperature used to heat the polymer in the extruder barrel may be, for example, at least about 300 °F, at least about 350 °F, at least about 400 °F, or at least about 420 °F. The maximum temperature of the extruder barrel may be, for example, between about 400 °F and about 630 °F. For instance, the maximum temperature of the extruder barrel may be between about 410 °F and about 600 °F, between about 410 °F and about 580 °F, between about 420 °F and about 550 °F, between about 420 °F and about 480 °F, or between about 420 °F and about 500 °F. In certain embodiments of the present disclosure, the maximum temperature of the extruder barrel may be greater than about 400 °F, greater than about 420 °F, greater than about 440 °F, greater than about 460 °F, greater than about 480 °F, or greater than about 500 °F. In other embodiments, the maximum temperature of the extruder barrel may be less than about 630 °F, less than about 550 °F, less than about 500 °F, or less than about 450 °F. In some embodiments, the maximum temperature of the extruder barrel is at least about 10 °F lower, at least about 20 °F lower, at least about 30 °F lower, or at least about 40 °F lower than the temperature of the die body. Other ranges and values of temperatures of the extruder barrel are also possible.

The process air temperature may also be varied. In some embodiments of the present disclosure, the process air temperature may be between about 400 °F and about 630 °F. For instance, the process air temperature may be between about 410 °F and about 600 °F, between about 410 °F and about 580 °F, between about 420 °F and about 550 °F, between about 440 °F and about 530 °F, or between about 420 °F and about 500 °F. Other ranges and values of process air temperatures are also possible.

In some embodiments of the present disclosure, it may be desirable to vary the process air volume. As described above, the process air is the heated air on either side of the die tip where the fibers are formed. This heated air (typically the same temperature as the die tip) impinges the fibers and helps attenuate the fibers to the final fiber size. It is believed that, in some embodiments, as the air volume increases, the fiber diameter can decrease. The process air volume can be selected as appropriate. In some embodiments, the process air volume may be between about 1,000 pounds/hour-meter (lbs/hr·m) and about 4,000 lbs/hr·m. For instance, the process air volume may be between about 1,500 lbs/hr·m and about 3,800 lbs/hr·m, between about 2,500 lbs/hr·m and about 3,750 lbs/hr·m, or between about 3,000 lbs/hr·m and about 3,500 lbs/hr·m. Other ranges and values of process air volumes are also possible.

The quench air temperature may also be varied. In some embodiments of the present disclosure, the quench air temperature may be between about 0 °F and about 200 °F. For instance, the quench air temperature may be between about 0 °F and about 150 °F, between about 0 °F and about 100 °F, between about 0 °F and about 75 °F, between about 0 °F and about 50 °F, between about 0 °F and about 30 °F, or between about 0 °F and about 20 °F. Other ranges and values of quench air temperatures are also possible.

In some embodiments of the present disclosure, it may be desirable to vary the quench air volume. In some embodiments, the quench air volume may be between about 0 pounds/hour (lbs/hr) and about 750 lbs/hr. For instance, the quench air volume may be between about 0 lbs/hr and about 500 lbs/hr, between about 0 lbs/hr and about 250 lbs/hr, or between about 0 lbs/hr and about 150 lbs/hr. Other ranges and values of quench air volumes are also possible.

The size of the die outlets (e.g., holes) and number of outlets per inch for the die can generally be selected as desired. In some embodiments of the present disclosure, the die can have about 35 holes per inch with 0.0125" holes. In certain embodiments, the die can have about 70 holes per inch with 0.007" holes. In some embodiments, the die can have from about 25 holes per inch to about 250 holes per inch. In certain cases, the die may include about 35 holes per inch or greater, about 50 holes per inch or greater, or about 70 holes per inch or greater. Other dies can optionally be used.

In some embodiments of the present disclosure, the distance from the die tip to the collector may be varied. The distance from the die tip to the collector may be, for example, between about 3 inches and about 80 inches. For instance, the distance from the die tip to the collector may be between about 3 inches and about 50 inches, between about 4 inches and about 40 inches, between about 5 inches and about 25 inches, or between about 6 inches and about 15 inches. Other ranges and values of distances from the die tip to the collector are also possible.

The vacuum level created by the suction box can be selected as appropriate. In some embodiments of the present disclosure, the vacuum level may be between about 1 inches of water and about 60 inches of water. For instance, the vacuum level may be between about 10 inches of water and about 50 inches of water, between about 20 inches of water and about 40 inches of water, between about 20 inches of water and about 30 inches of water, or between about 30 inches of water and about 40 inches of water.

The line speed at which the collector belt moves can be selected as desired to form a fiber web. In some embodiments of the present disclosure, the collector belt may move at a line speed between about 1 ft/min and about 400 ft/min. For instance, the collector belt may move at a line speed between about 10 ft/min and about 200 ft/min, between about 50 ft/min and about 150 ft/min, between about 50 ft/min and about 100 ft/min, or between about 75 ft/min and about 150 ft/min.

It should be understood that the values and ranges of the parameters described above can be used in different combinations to control fiber formation during an extrusion process. For example, in some embodiments a relatively low dwell time and a relatively low throughput may be used to form fine fibers. For instance, in one set of embodiments of the present disclosure, a method may include subjecting the polymeric material to a dwell time of less than about 30 minutes and a throughput of less than about 85 lbs/hr. In another set of embodiments, the polymeric material may have a dwell time of less than about 50 minutes and a throughput of less than about 55 lbs/hr. In some embodiments, using these or other parameters, fiber webs having relatively low surface densities of particles can be formed as described in more detail below.

In some embodiments, varying the above-noted parameters during an extrusion process, and/or using one or more additives described herein, may result in essentially none or relatively low amounts of polymer degradation during fiber formation. In some cases, such processes can be used to form fine fibers, such as ones having a diameter in one of the ranges described herein (e.g., an average diameter between about 0.1 and about 1.5 microns, or between about 0.1 and about 0.6 microns). Without wishing to be bound by any theory, the inventors believe that subjecting the polymer material used to form the fibers to relatively high temperatures and pressures for extended periods of time in an extrusion system can cause the polymeric material to degrade. Degradation may involve chain scission, i.e., shortening of the polymer chains to produce lower molecular weight polymers, and/or other forms of decomposition (e.g., chemical decomposition, thermal decomposition, ionization). As a result of polymer degradation, small polymeric particles may be formed. These particles may have the same chemical composition as the polymeric material used to form the fibers (but having a lower molecular weight), or may be a derivative of the polymeric material used to form the fibers. The particles may be associated with the fiber web in various configurations. For instance, the particles may reside on the surface of the fibers, on the surface of the fiber web, in the center of the fiber web, or in combinations thereof. As noted above, as the amount of degraded polymer increases, less fiber is produced per unit of polymer. For fiber webs used for filtration, for example, this occurrence is not desirable as it may result in increased basis weight in order to achieve the same level of performance as fiber webs without degraded polymer, all other factors being equal.

The shape and size of the polymeric particles formed may vary, and in some cases, the particles can even agglomerate to form larger particles. It should be understood that the polymeric particles described herein are different from fibers. The polymeric particles are non-fibrous, and generally have an aspect ratio (i.e., a length to largest cross-sectional dimension) of less than 50:1 and a largest cross-sectional dimension of at least 0.2 mm. In some embodiments, a particle may have a largest cross-sectional dimension of about 0.2 mm or greater, about 0.5 mm or greater, about 1.0 mm or greater, about 1.5 mm or greater, about 2.0 mm or greater, about 2.5 mm or greater, about 3.0 mm or greater, about 3.5 mm or greater, about 4.0 mm or greater, about 4.5 mm or greater, about 5.0 mm or greater, about 5.5 mm or greater, about 6.0 mm or greater, about 6.5 mm or greater, about 7.0 mm or greater, about 7.5 mm or greater, about 8.0 mm or greater, about 8.5 mm or greater, about 9.0 mm or greater, about 9.5 mm or greater, or about 10.0 mm or greater. Other values and ranges of particle size are also possible.

In certain embodiments, the average molecular weight of the particles formed during a fiber extrusion process may be less than about 1/2 the average molecular weight of the polymer used to form the fibers. For instance, the average molecular weight of the particles formed during a fiber extrusion process may be less than about 1/8, less than about 1/64, or less than about 1/200 the average molecular weight of the polymer used to form the fibers. Other values of molecular weight of the particles associated with a fiber web are also possible.

In some embodiments, a fiber web described herein may include a relatively low number of or essentially no particles on its surface. The amount of particles may be measured by determining the surface density of particles on the fiber web, i.e., the number of particles on a surface of the fiber web per unit area of the fiber web surface. For instance, a fiber web may have a surface density of particles of less than about 12.0 particles/inch², less than about 11.5 particles/inch², less than about 11.0 particles/inch², less than about 10.5 particles/inch², less than about 10.0 particles/inch², less than about 9.5 particles/inch², less than about 9.0 particles/inch², less than about 8.5 particles/inch², less than about 8.0 particles/inch², less than about 7.5 particles/inch², less than about 7.0 particles/inch², less than about 6.5 particles/inch², less than about 6.0 particles/inch², less than about 5.5 particles/inch², less than about 5.0 particles/inch², less than about 4.5 particles/inch², less than about 4.0 particles/inch², less than about 3.5 particles/inch², less than about 3.0 particles/inch², less than about 2.7 particles/inch², less than about 2.5 particles/inch², less than about 2.2 particles/inch², less than about 2.0 particles/inch², less than about 1.8 particles/inch², less than about 1.6 particles/inch², less than about 1.5 particles/inch², less than about 1.3 particles/inch², less than about 1.0 particles/inch², less than about 0.8 particles/inch², less than about 0.5 particles/inch², or less than about 0.3 particles/inch², wherein each of the particles has a largest cross-sectional dimension of one of the ranges or values described above. For example, in one particular embodiment, a fiber web has a surface density of particles of less than about 3.0 particles/inch², wherein each of the particles has a largest cross-sectional dimension of between about 0.2 mm or greater. In this embodiment, even though the fiber web may include some particles having a largest cross-sectional dimension smaller than about 0.2 mm, these particles are not accounted for in calculating the surface density of particles. In another embodiment, a fiber web has a surface density of particles of less than about 3.0 particles/inch², wherein each of the particles has a largest cross-sectional dimension of about 1.0 mm or greater. In this embodiment, even though the fiber web may include some particles having a largest cross-sectional dimension smaller than about 1.0 mm, these particles are not accounted for in calculating the surface density of particles. Other surface densities of particles in a particular size range or value are also possible.

The number of particles per area of fiber web can be determined as follows. A sample of fiber web can be layered together with carbon paper and a white sheet of standard copy paper, where the carbon paper is positioned between the fiber web and the copy paper. The composite structure can be placed in a continuous belt press where the following conditions are employed: a line speed of 2.5 m/min, a pressure of 6 bar, and a temperature of about 68 °F - 80 °F (room temperature). After exposure to these conditions, the degraded polymer particles, if present, may lie at an elevated position compared to the fibers, and appear as small "dots" on the underlying copy paper. If a darker image is needed for detection, the copy paper can be photocopied with a standard copier to darken the carbon image. This copy paper image can be scanned using standard imaging software, and software (e.g., ImageJ software available for download at http://rsbweb.nih.gov/ij/) can be used to determine the number of "dots" on the image. These "dots" may be measured in pixels, and each pixel can be correlated to a certain size to determine the size and number of particles. For instance, 1 pixel may correspond to 0.2646 mm, so a "dot" having a size of 1 pixel on the image may correspond to 1 particle having a largest dimension of 0.2646 mm; a "dot" having a size of 4 pixels on the image may correspond to 1 particle having a largest dimension of 1.1 mm. Pixel sizes may vary depending on the imaging hardware and/or software used. To calculate a surface density of particles, wherein each of the particles has a largest cross-sectional dimension of, for example, about 1.0 mm or greater, only the "dots" having a size of at least 4 pixels (e.g., a largest cross-sectional dimension of about 1.0 mm or greater) would be counted. This number would be divided by the area of the fiber web used for counting the particles to determine the surface density of particles. In this particular instance, even though the fiber web may include some particles having a largest cross-sectional dimension smaller than about 1.0 mm, these particles are not accounted for for the purpose of this particular calculation.

In some embodiments, fiber webs having a value or range of surface density of particles described above can also have one or more of the values and ranges of the features and performance characteristics described below.

In some embodiments, at least 5% (e.g., at least 7%, at least 10%, at least 15%, at least 20%, at least 25%, at least 50%, at least 60%, or at least 75%) of the fibers in a layer of a fiber web extend a distance of at least 0.3 microns in a direction substantially perpendicular to a surface of the layer,

A fiber web described herein may be formed of fibers having an average diameter between about 0.1 microns and about 1.5 microns. For instance, the fiber web may include fibers (e.g., meltblown fibers) having an average diameter of between about 0.1 microns and about 1.3 microns, between about 0.1 microns and about 1.2 microns, between about 0.1 microns and about 1.0 microns, between about 0.25 microns and about 1.0 microns, between about 0.1 microns and about 0.8 microns, between about 0.1 microns and about 0.7 microns, between about 0.1 microns and about 0.6 microns, between about 0.1 microns and about 0.5 microns, or between about 0.1 microns and about 0.4 microns. In some embodiments, the average diameter of the fibers (e.g., meltblown fibers) in a fiber web may be about 1.5 microns or less, about 1.4 microns or less, about 1.3 microns or less, about 1.2 microns or less, about 1.1 microns or less, about 1.0 microns or less, about 0.9 microns or less, about 0.8 microns or less, about 0.7 microns or less, about 0.6 microns or less, about 0.5 microns or less, about 0.4 microns or less, or about 0.3 microns or less. In other embodiments, the average diameter of the fibers (e.g., meltblown fibers) in a fiber web may be greater than about 0.2 microns, greater than about 0.4 microns, greater than about 0.6 microns, greater than about 0.8 microns, greater than about 1.0 microns, or greater than about 1.2 microns. As used herein, fiber diameter is measured using scanning electron microscopy.

A particular fiber used in a fiber web described herein (e.g., a meltblown fiber having an average fiber diameter of about 1.0 microns) generally has a standard deviation of fiber diameter associated with it. The standard deviation of fiber diameter may depend on the particular process used to form the fiber. For example, the standard deviation of fiber diameter for meltblown fibers is generally greater than about 0.20 microns (e.g., typically greater than about 0.70 microns), whereas the standard deviation of fiber diameter for electrospun fibers is generally less than about 0.20 microns (e.g., typically less than about 0.10 microns).

In some embodiments, the standard deviation of fiber diameter for a fiber described herein (e.g., meltblown fibers) may be greater than about 0.15 microns, greater than about 0.20 microns, greater than about 0.25 microns, greater than about 0.30 microns, greater than about 0.35 microns, greater than about 0.40 microns, greater than about 0.45 microns, greater than about 0.50 microns, greater than about 0.55 microns, greater than about 0.60 microns, greater than about 0.65 microns, greater than about 0.70 microns, greater than about 0.75 microns, or greater than about 0.80 microns. In certain embodiments, the standard deviation of fiber diameter for a fiber described herein (e.g., meltblown fibers) may be less than about 1.0 microns, less than about 0.90 microns, less than about 0.80 microns, less than about 0.70 microns, less than about 0.60 microns, less than about 0.50 microns, less than about 0.40 microns, less than about 0.30 microns, or less than about 0.20 microns. Other ranges are also possible. Combinations of the above-noted ranges are also possible (e.g., a standard deviation of greater than about 0.15 microns and less than about 0.70 microns). The standard deviation may be calculated using a total number of samples of at least 18 in some embodiments. In other embodiments, the total number of samples used to calculate standard deviation may be at least 25, at least 50, or at least 100.

In some cases, a fiber described herein (e.g., meltblown fibers) has a particular ratio of average fiber diameter to standard deviation of fiber diameter. For instance, a fiber having an average diameter of 0.38 microns with a standard deviation of 0.53 microns would have a ratio of average fiber diameter to standard deviation of fiber diameter of 1:1.4. In some embodiments, a fiber described herein may have a ratio of average fiber diameter to standard deviation of fiber diameter of less than about 5.0:1.0 (e.g., 4.5:1.0), less than about 4.0:1.0, less than about 3.0:1.0, less than about 2.0:1.0, or less than about 1.0:1.0 (e.g., 0.7:1.0). In certain embodiments, a fiber described herein may have a ratio of average fiber diameter to standard deviation of fiber diameter of greater than about 0.5:1.0, greater than about 0.6:1.0, greater than about 0.7:1.0, greater than about 0.8:1.0, greater than about 0.9:1.0, greater than about 1.0:1.0, greater than about 1.5:1.0. Other ranges are also possible. Combinations of the above-noted ranges are also possible (e.g., a ratio of less than about 5.0:1.0 and greater than about 0.7:1.0).

The fiber web can generally have any suitable thickness. In some embodiments, the fiber web has a thickness between about 0.0005 inches and about 0.040 inches. For instance, the thickness of the fiber web may be between about 0.001 inches and about 0.030 inches, between about 0.001 inches and about 0.020 inches, between about 0.002 inches and about 0.010 inches, or between about 0.002 inches and about 0.020 inches. In some instances, the thickness of the fiber web may be less than about 0.040 inches, less than about 0.030 inches, less than about 0.020 inches, or less than about 0.010 inches. In other instances, the thickness of the fiber web may be greater than about 0.0010 inches, greater than about 0.0050 inches, greater than about 0.010 inches, greater than about 0.020 inches, or greater than about 0.030 inches. As referred to herein, thickness is determined according to the standard ASTM D1777.

In certain embodiments, the fiber webs described herein have a relatively high consistency (low variability) of thickness across the fiber web. For instance, the variability of thickness across the fiber web may be about 6.0 standard deviations or less, about 5.5 standard deviations or less, about 5.0 standard deviations or less, about 4.5 standard deviations or less, about 4.0 standard deviations or less, about 3.5 standard deviations or less, about 3.0 standard deviations or less, about 2.5 standard deviations or less, about 2.0 standard deviations or less, about 1.5 standard deviations or less, about 1.0 standard deviations or less, or about 0.5 standard deviations or less. Other values of thickness variability are also possible. The variability of thickness may be determined by taking a statistically significant number of measurements across the fiber web.

The basis weight of the fiber web can typically be selected as desired. In some embodiments, the basis weight of the fiber web may be between about 1.0 g/m² and about 100 g/m². For instance, the basis weight of the fiber web may be between about 1.0 g/m² and about 70 g/m² between about 2.0 g/m² and about 70 g/m², between about 3.0 g/m² and about 30 g/m² between about 1.0 g/m² and about 50 g/m², between about 1.0 g/m² and about 30 g/m² between about 2.0 g/m² and about 30 g/m², between about 3.0 g/m² and about 30 g/m², or between about 3.0 g/m² and about 20 g/m². In some embodiments, the basis weight of the fiber web is greater than about 1 g/m² (e.g., greater than about 2.0 g/m², greater than about 3.0 g/m², greater than about 4.0 g/m², greater than about 5.0 g/m², greater than about 10 g/m², greater than about 25 g/m²), and/or less than about 100 g/m² (e.g., less than about 90 g/m², less than about 75 g/m², less than about 30 g/m², less than about 20 g/m², less than about 10 g/m²). As referred to herein, basis weight is determined according to ASTM D3776.

In certain embodiments, the fiber webs described herein have a relatively high consistency (low variability) of basis weight across the fiber web. For instance, the variability of basis weight across the fiber web may be about 6.0 standard deviations or less, about 5.5 standard deviations or less, about 5.0 standard deviations or less, about 4.5 standard deviations or less, about 4.0 standard deviations or less, about 3.5 standard deviations or less, about 3.0 standard deviations or less, about 2.5 standard deviations or less, about 2.0 standard deviations or less, about 1.5 standard deviations or less, about 1.0 standard deviations or less, or about 0.5 standard deviations or less. Other values of basis weight variability are also possible. The variability of basis weight may be determined by taking a statistically significant number of measurements across the fiber web.

In certain embodiments, the fiber webs described herein may have a relatively high surface area. In certain embodiments according to the present invention, a fiber web may have a surface area between between about 2.0 m²/g and about 6.0 m²/g, or between about 2.5 m²/g and about 6.0 m²/g. In some cases, a fiber web has a surface area of about 2.0 m²/g or greater, about 2.1 m²/g or greater, 2.2 m²/g or greater, about 2.3 m²/g or greater, about 2.4 m²/g or greater, about 2.5 m²/g or greater, about 2.6 m²/g or greater, about 2.7 m²/g or greater, about 2.8 m²/g or greater, 2.9 m²/g or greater, or about 3.0 m²/g or greater. As determined herein, surface area is measured through use of a standard BET surface area measurement technique. The BET surface area is measured according to section 10 of Battery Council International Standard BCIS-03A, "Recommended Battery Materials Specifications Valve Regulated Recombinant Batteries", section 10 being "Standard Test Method for Surface Area of Recombinant Battery Separator Mat". Following this technique, the BET surface area is measured via adsorption analysis using a BET surface analyzer (e.g., Micromeritics Gemini III 2375 Surface Area Analyzer) with nitrogen gas; the sample amount is between 0.5 and 0.6 grams in a 3/4" tube; and, the sample is allowed to degas at 75 degrees C for a minimum of 3 hours.

The mean pore size of the fiber web may also vary. In some embodiments, a fiber web has a mean pore size between about 1 micron and about 30 microns. For instance, the mean pore size may be between about 1 micron and about 20 microns, between about 1 micron and about 15 microns, between about 5 microns and about 15 microns, between about 1 micron and about 10 microns, or between about 5 microns and about 15 microns. In certain embodiments, the mean pore size may be less than about 30 microns, less than about 25 microns, less than about 20 microns, less than about 15 microns, less than about 10 microns, or less than about 5 microns. In other embodiments, the mean pore size may be greater than about 5 microns, greater than about 10 microns, greater than about 15 microns, greater than about 20 microns, greater than about 25 microns, or greater than about 30 microns. Other values and ranges of mean pore size are also possible. As used herein, mean pore size is measured according to the standard ASTM F-316-80 Method B, BS6410, e.g., using a Capillary Flow Porometer made by Porous Materials Inc.

Typically, the fiber web is formed of one or more polymers. Exemplary polymers include polyolefins (e.g., polypropylenes), polyesters (e.g., polybutylene terephthalate, polybutylene naphthalate), polyamides (e.g., nylons), polycarbonates, polyphenylene sulfides, polystyrenes, polyurethanes (e.g., thermoplastic polyurethanes). Optionally, the polymer(s) may contain fluorine atoms. Examples of such polymers include PVDF and PTFE. Examples of specific polymers that may be used include a polypropylene manufactured by LyondellBasell (MF650Y), a polypropylene manufactured by Total Petrochemicals (3962), a polypropylene manufactured by Exxon (PP3546G and ACHV6936G1 Metocene PP), a polypropylene manufactured by Borealis (HL512FB), a polyester (PBT) manufactured by Ticona (HB85151M1 CX2008) and a nylon manufactured by BASF (Ultramid B3SQ661). Other polymers suitable for use in an extrusion process can also be used.

In some embodiments, the fiber web includes one or more additives such as a binder, a lubricant, a slip agent, a surfactant, a coupling agent, a crosslinking agent, amongst others. In certain instances, one or more additives can be used to reduce or eliminate the number of polymeric particles formed on or in a fiber web.

Generally, the fiber web includes a small weight percentage of an additive. For example, the fiber web may include less than about 10%, less than about 8%, less than about 6%, less than about 5%, or less than about 4% of an additive. In some cases, the fiber web may include between about 1% and about 10%, between about 1% and about 8%, between about 1% and about 5% of an additive, or between about 1% and about 2.5% of an additive. In certain embodiments, the fiber web may include less than about 5%, less than about 3%, less than about 2%, or less than about 1% of a fatty acid additive as described below. In some embodiments, the additive may be added to the polymer material used to form the fibers when the polymeric material is in a molten (e.g., melted) state. In other embodiments, the additive coats the fibers after the fibers have been formed.

In some embodiments, a fiber web may include an additive (e.g., a slip agent or other type of additive) in the form of a lipid. In some cases, the additive comprises a fatty acid (e.g., a saturated fatty acid, an unsaturated fatty acid, a mono-unsaturated fatty acid, a poly-unsaturated fatty acid). In certain embodiments, the fatty acid includes an amide group (e.g., a fatty acid amide). Non-limiting examples of fatty acid amides include stearamide, behenamide, erucamide, N-(2-hdriethyl) erucamide, lauramide, N,N'-ethylene-bis-oleamide, N,N'-ethylene bissteamide, oleamide, oleyl palmitamide, stearyl erucamide, tallow amide, arachidonylethanolamide, N-arachidonylmaleimide, mixtures thereof, and derivatives thereof.

Examples of specific additives that may be used include an additive provided by Standridge Color Corp., having a supplier part no.: 22686, and an additive containing provided by Standridge Color Corp., having a supplier part no. 10SAM1044.

In certain embodiments, the additive is in the form of a fatty acid having a Cₙ (carbon) chain, where n is an integer. In some cases, n is 2 or greater, 4 or greater, 6 or greater, 8 or greater, 10 or greater, 12 or greater, 14 or greater, 16 or greater, 18 or greater, 20 or greater, 22 or greater, 24 or greater, 26 or greater, 28 or greater, 30 or greater, 32 or greater, 34 or greater, 36 or greater, 38 or greater, or 40 or greater. In other cases, n is less than or equal to 50, less than or equal to 45, less than or equal to 40, less than or equal to 35, less than or equal to 40, less than or equal to 35, less than or equal to 30, less than or equal to 25, less than or equal to 20, less than or equal to 15, less than or equal to 10, or less than or equal to 5.

The fiber webs described herein may have various performance characteristics. In some cases, the fiber webs have performance characteristics that enable them to be suitable for use as filter media.

In some embodiments, methods described herein for forming meltblown fibers can result in a fiber web having a relatively low air permeability. For instance, the air permeability of a fiber web may be less than about 1,800 ft³/min/ft² (CFM), less than about 1,500 CFM, less than about 1,300 CFM, less than about 1,000 CFM, less than about 900 CFM, less than about 800 CFM, less than about 750 CFM, less than about 700 CFM, less than about 600 CFM, less than about 500 CFM, less than about 400 CFM, less than about 300 CFM, less than about 200 CFM, less than about 100 CFM, or less than about 50 CFM. In general, however, the air permeability of the fiber web can vary between about 10 CFM and about 1800 CFM (e.g., between about 10 CFM and about 1,500 CFM, between about 10 CFM and about 1,000 CFM, between about 10 CFM and about 750 CFM, between about 40 CFM and about 750 CFM, between about 10 CFM and about 600 CFM, between about 10 CFM and about 500 CFM, between about 10 CFM and about 400 CFM, between about 10 CFM and about 300 CFM, between about 10 CFM and about 200 CFM, between about 10 CFM and about 100 CFM, or between about 10 CFM and about 50 CFM). Other ranges are also possible. As used herein, air permeability is measured according to the standard ASTM D737-75.

The fiber webs described herein may have different ranges of NaCl particle filtration efficiencies. The NaCl particle filtration efficiency is [1-(C/C₀)]*100%, where C is the NaCl particle concentration after passage through the fiber web and C₀ is the NaCl particle concentration before passage through the filter. To measure NaCl particle filtration efficiency, a 100 cm² surface area of the fiber web can be tested with NaCl (sodium chloride) particles having a 0.26 micron mass mean diameter with a geometric standard deviation less than 1.83, a concentration of 15 to 20 mg/cm³, and a face velocity of 5.3 cm/s by a TSI 8130 CertiTest(TM) automated filter testing unit from TSI, Inc. equipped with a sodium chloride generator. The instrument measures a pressure drop (e.g., an airflow resistance) across the fiber web and the resultant penetration value on an instantaneous basis at a flow rate less than or equal to 115 liters per minute (lpm). Instantaneous readings can be defined as 1 pressure drop/penetration measurement. This test is described in ASTM D2 986-91.

A fiber web described herein may have a NaCl particle filtration efficiency between about 0.0001% and about 99.97%. For instance, the NaCl particle filtration efficiency may be between about 0.001% and about 99.97%, between about 0.01% and about 99.97%, between about 0.1% and about 99.97%, between about 1% and about 99.97%, between about 10.0% and about 99.97%, between about 40.0% and about 99.97%, between about 60.0% and about 99.97%, or between about 85.0% and about 99.97%. In some cases, the NaCl particle filtration efficiency is greater than about 10.0%, greater than about 20.0%, greater than about 30.0%, greater than about 40.0%, greater than about 50.0%, greater than about 60.0%, greater than about 70.0%, greater than about 80.0%, greater than about 90.0%, greater than about 95.0%, greater than about 97.0%, greater than about 98.0%, greater than about 99.0%, greater than about 99.5%, greater than about 99.9%, or greater than about 99.97%. Other ranges and values of NaCl particle filtration efficiency are also possible.

In some cases, a fiber web described herein may have an airflow resistance between about 0.1 mm H₂O and about 50.0 mm H₂O. For instance, the air flow resistance may be between about 0.1 mm H₂O and about 40.0 mm H₂O, between about 0.1 mm H₂O and about 30.0 mm H₂O, between about 0.1 mm H₂O and about 20.0 mm H₂O, between about 0.1 mm H₂O and about 10.0 mm H₂O, between about 0.3 mm H₂O and about 5.0 mm H₂O, between about 0.3 mm H₂O and about 3.5 mm H₂O, between about 0.3 mm H₂O and about 3.0 mm H₂O, between about 0.1 mm H₂O and about 2.5 mm H₂O, or between about 0.1 mm H₂O and about 2.0 mm H₂O. In some cases, the air flow resistance of a fiber web is less than about 50.0 mm H₂O, less than about 40.0 mm H₂O, less than about 30.0 mm H₂O, less than about 20.0 mm H₂O, less than about 10.0 mm H₂O, less than about 5.0 mm H₂O, or less than about 2.5 mm H₂O. In other cases, the air flow resistance of a fiber web is greater than about 1.0 mm H₂O, greater than about 2.5 mm H₂O, greater than about 5.0 mm H₂O, greater than about 10.0 mm H₂O, greater than about 20.0 mm H₂O, greater than about 30.0 mm H₂O, or greater than about 40.0 mm H₂O, Other ranges and values of air flow resistance are also possible. As used herein, air flow resistance is measured according to the standard ASTM D2 986-91 as described above.

It should be understood that the fiber webs described herein having the values and ranges of the features and performance characteristics described above may be formed using different combinations of the parameters described above to control fiber formation during an extrusion process. For example, in some embodiments, a method involving subjecting the polymeric material used to form the fibers to a dwell time of less than about 85 minutes, and using an extruder barrel having an inner diameter of about 4 inches or less, may lead to fibers having small diameters (e.g., average diameter of about 1.0 microns or less, about 0.8 microns or less, or about 0.6 microns or less), fiber webs having relatively high surface areas (e.g., about 1.8 m²/g or greater, about 2.0 m²/g or greater, or about 2.2 m²/g or greater), and/or to fiber webs having relatively low amounts of polymer degradation (e.g., a surface density of polymeric particles of less than about 5.0 particles/in², less than about 3.0 particles/in², less than about 2.0 particles/in², less than about 1.6 particles/in², less than about 1.0 particles/in², or less than about 0.8 particles/in², less than about 0.5 particles/in², or less than about 0.3 particles/in², wherein each of the particles has a largest cross-sectional dimension of 1.0 mm or greater). In other embodiments, a method of forming fibers involving subjecting the polymeric material used to form the fibers to a processing space having a volume less than about 25,000 cm³, less than about 15,000 cm³, or less than about 9,000 cm³ may lead to fibers and/or fiber webs having these characteristics.

It should also be understood that the fiber webs described herein may have a single layer or multiple layers. In embodiments in which a fiber web includes more than one layer, in some cases each layer of the fiber web may be formed by a process described herein. In other cases, at least one layer, or at least two layers, of the fiber web may be formed by a process described herein. Likewise, in embodiments in which a fiber web includes more than one layer, in some cases each layer of the fiber web may have one or more characteristics (e.g., surface density of particles, fiber diameter, standard deviation of fiber diameter, thickness, variability of thickness across the fiber web, basis weight, variability of basis weight across the fiber web, surface area, mean pore size, polymer type, presence of an additive, or a performance characteristic) in one or more of the ranges described herein. In other cases, at least one layer, or at least two layers of the fiber web, may have one or more characteristics (e.g., surface density of particles, fiber diameter, standard deviation of fiber diameter, thickness, variability of thickness across the fiber web, basis weight, variability of basis weight across the fiber web, surface area, mean pore size, polymer type, presence of an additive, or a performance characteristic) in one or more of the ranges described herein.

In certain embodiments, a fiber web described herein may be combined with one or more other components such as a substrate and/or a scrim, optionally with an adhesive. Examples of substrates, scrims and adhesives are described in U.S. Publication No. 2009/0120048, filed November 07, 2008, and entitled "Meltblown Filter Medium".

In some cases, a fiber web or a composite including a fiber web can be charged. In general, any of a variety of techniques can be used to charge the fiber web and or a composite including the fiber web to form an electret web. Examples include AC and/or DC corona discharge. In some embodiments, the composite is subjected to a discharge of at least 1 kV/cm (e.g., at least 5 kV/cm, at least 10 kV/cm), and/or at most 30 kV/cm (e.g., at most 25 kV/cm, at most 20 kV/cm). For example, in certain embodiments, the composite can be subjected to a discharge of from 1 kV/cm to 30 kV/cm (e.g., from 5 kV/cm to 25 kV/cm, from 10 kV/cm to 20 kV/cm). Exemplary processes are disclosed, for example, in U.S. Pat. No. 5,401,446.

In some embodiments, a fiber web described herein can be a part of a filter element. Examples of filter elements include gas turbine filter elements, heavy duty air filter elements, automotive air filter elements, HVAC air filter elements, HEPA filter elements, vacuum bag filter elements, fuel filter elements, and oil filter elements. Such filter elements can be incorporated into corresponding filter systems (gas turbine filter systems, heavy duty air filter systems, automotive air filter systems, HVAC air filter systems, HEPA filter systems, vacuum bag filter systems, fuel filter systems, and oil filter systems). Vacuum filter bag systems are commonly used in home vacuum cleaners. In such embodiments, a filter medium can optionally be prepared by coating a paper with the meltblown material. In certain embodiments, a filter medium can be prepared using a wet laid or dry laid product (e.g., cellulose, polymer, glass). A filter medium can optionally be pleated into any of a variety of configurations (e.g., panel, cylindrical). Examples of filter media are described in more detail in U.S. Publication No. 2009/0120048, filed November 07, 2008, and entitled "Meltblown Filter Medium".

The following examples are exemplary and not intended as limiting.

### EXAMPLES 1-10

Examples 1-10 (Examples 1-7 not forming part of the invention) show that various process parameters of an extrusion process can be varied to form fiber webs having small fiber diameters, high surface area, low air permeabilities, and/or low levels of polymer degradation according to certain embodiments described herein.

A total of 80 experiments were conducted in which different fiber webs were formed with either polypropylene or polyester (polybutyleneterephthalate) fibers using a process similar to the one shown in FIG. 1, while varying various process conditions including extruder barrel inner diameter, die body temperature, and polymer throughput. Performance characteristics and physical properties of the resulting fiber webs including air permeability, level of polymer degradation (e.g., surface density of particles), surface area, and fiber size were measured, and the values were compiled and input into modeling software, where mathematical modeling of these properties was performed. The models were refined (through reduction) until an acceptable accountability of the combined effect was obtained. A response calculation for each of the performance characteristics and physicals properties was determined.

The resulting, non-coded, mathematical models were then placed into an Excel spreadsheet, where a simple mathematical equation function was utilized to render the predicted physical property values of fiber webs that may be produced using different processing conditions (e.g., varying the values for extruder barrel inner diameter, die body temperature and polymer throughput). The results of the calculations are shown in Tables 1-3.

For each of the Examples shown in Tables 1-3, the following processing conditions would be used: extruder temperature profile (ramping) of 300 °F, 325 °F, 350 °F, 375 °F, 400 °F, 425 °F, 450 °F; the process air temperature being the same as that of the die body temperature; a process air setting of 3150 lbs/hr; a die to collector distance of 8.0 inches; a quench air rate of 225 lbs/hr; and a vacuum level of 17,500 ft³.

**Table 1**

| | **Comparative Example 1** | **Example 1**** | **Example 2**** | **Example 3**** |
|---|---|---|---|---|
| Extruder Barrel Inner Diameter (inches) | 5 | 2 | 1 | 1 |
| Extruder Barrel Length (inches) | 150 | 60 | 30 | 30 |
| Conduit Diameter (inches) | 1.5 | 1 | 0.75 | 0.75 |
| Conduit Length (inches) | 144 | 144 | 144 | 144 |
| Polymer Type | Polypropylene (PP) | PP | PP | PP |
| Polymer Throughput (lb/hr) | 30 | 58 | 61 | 102 |
| Die Body Temp (°F) | 470 | 510 | 510 | 530 |
| Dwell Time (min) | 157 | 13 | 9 | 5 |
| Volume of processing space (cm³) | 25459 | 6300 | 4541 | 4541 |
| Air Permeability (ft³/min/ft²) | 409 | 409 | 409 | 409 |
| Surface Area (m²/g) | 1.14 | 1 | 0.95 | - |
| Surface density of particles* (particles/in²) | 3.29 | 0 | 0 | 0.25 |
| Fiber Diameter (microns) | 0.95 | 1.2 | 1.28 | 1.44 |

| | | | | |
|---|---|---|---|---|
| * The particles refer to ones having a largest cross-sectional dimension of 1.0 mm or greater. ** Reference Example, does not form part of the invention. | | | | |

Examples 1-3 show that by reducing the extruder barrel inner diameter, extruder barrel length and conduit diameter, and increasing the polymer throughput, the dwell times of the polymer in the processing space can be reduced. The surface density of particles of degraded polymer in fiber webs produced by processes under such conditions would be reduced compared to that of Comparative Example 1, where the dwell time is relatively higher. Examples 1-3 also show that by decreasing the volume of the processing space (e.g., by reducing the extruder barrel length and conduit diameter), relatively high throughputs can be used and can be used to form fiber media having similar performance characteristics (e.g., air permeability) as media formed by the processing conditions shown for Comparative Example 1 (e.g., lower throughputs but higher processing space volumes). Higher throughputs may result in lower manufacturing costs.

**Table 2**

| | **Comparative Example 2** | | **Example 5**** | **Example 6**** | **Example 7**** |
|---|---|---|---|---|---|
| Extruder Barrel Inner Diameter (inches) | 5 | 2 | 2 | 1 | 1 |
| Extruder Barrel Length (inches) | 150 | 60 | 60 | 30 | 30 |
| Conduit Diameter (inches) | 1.5 | 1 | 1 | 0.75 | 0.75 |
| Conduit Length (inches) | 144 | 144 | 144 | 144 | 144 |
| Polymer Type | Polypropylen e (PP) | PP | PP | PP | PP |
| Polymer Throughput (lb/hr) | 30 | 30 | 30 | 30 | 30 |
| Die Body Temp (°F) | 470 | 470 | 510 | 510 | 530 |
| Dwell Time (min) | 100 | 24 | 24 | 17 | 17 |
| Volume of processing space (cm³) | 25459 | 6300 | 6300 | 4541 | 4541 |
| Air Permeability (ft³/min/ft²) | 409 | 403 | 261 | 229 | 143 |
| Surface Area (m²/g) | 1.14 | 1.23 | 1.48 | 1.56 | 1.7 |
| Surface density of particles* (particles/in²) | 3.29 | 0.75 | 0.75 | 0 | 0 |
| Fiber Diameter (microns) | 0.95 | 1.13 | 0.96 | 0.96 | 0.84 |

| | | | | | |
|---|---|---|---|---|---|
| * The particles refer to ones having a largest cross-sectional dimension of 1.0 mm or greater. ** Reference Example, does not form part of the invention. | | | | | |

Examples 4-7 show that by reducing the extruder barrel inner diameter, extruder barrel length and conduit diameter, the dwell time of the polymer in the processing space can be reduced. The surface density of particles of degraded polymer in fiber webs produced by processes under such conditions would be reduced compared to that of Comparative Example 2, where the dwell time is relatively higher. The processing conditions shown in Examples 4-7 can also result in fiber webs having lower air permeabilities and higher surface areas. Smaller fiber diameters (Example 7) can also be produced.

**Table 3**

| | **Comparative Example 2** | **Example 8** | **Example 9** | **Example 10** |
|---|---|---|---|---|
| Extruder Barrel Inner Diameter (inches) | 5 | 1.5 | 1.5 | 1.5 |
| Extruder Barrel Length (inches) | 150 | 45 | 45 | 45 |
| Conduit Diameter (inches) | 1.5 | 0.75 | 0.75 | 0.75 |
| Conduit Length (inches) | 144 | 144 | 144 | 144 |
| Polymer Type | Polypropylene (PP) | PP | PP | PP |
| Polymer Throughput (lb/hr) | 30 | 30 | 15 | 15 |
| Die Body Temp (°F) | 470 | 600 | 550 | 560 |
| Dwell Time (min) | 100 | 18 | 36 | 36 |
| Volume of processing space (cm³) | 25459 | 4862 | 4862 | 4862 |
| Air Permeability (ft³/min/ft²) | 409 | ∼89 | 69 | 46 |
| Surface Area (m²/g) | 1.14 | 2.13 | 2.07 | 2.14 |
| Surface density of particles* (particles/in²) | 3.28 | 0.30 | 0.53 | 0.53 |
| Fiber Diameter (microns) | 0.96 | 0.50 | 0.67 | 0.60 |

| | | | | |
|---|---|---|---|---|
| * The particles refer to ones having a largest cross-sectional dimension of 1.0 mm or greater. | | | | |

Examples 8-10 show that by reducing the extruder barrel inner diameter, extruder barrel length and conduit diameter, the dwell time of the polymer in the processing space can be reduced. The surface density of particles of degraded polymer in fiber webs produced by processes under such conditions would be reduced compared to that of Comparative Example 2, where the dwell time is relatively higher. The processing conditions shown in Examples 8-10 can also result in fiber webs having lower air permeabilities, higher surface areas, and smaller fiber diameters.

## Claims

1. A fiber web comprising:
a plurality of meltblown fibers having an average fiber diameter between about 0.1 microns and about 1.5 microns, wherein the fiber web has:
an air permeability measured according to the standard ASTM D737-75 between about 0.283 m³/min (10 CFM) and about 51.0 m³/min (1800 CFM);
a surface area greater than about 2.0 m²/g, wherein the surface area is measured using a BET surface analyzer according to section 10 of Battery Council International Standard BCIS-03A;
a basis weight determined according to ASTM D3776 between about 1.0 g/m² and about 100 g/m²; and
a thickness determined according to the standard ASTM D 1777 between about 0.0127 mm (0.0005 inches) and about 1.016 mm (0.04 inches).

2. The fiber web of claim 1, wherein the fiber web has
a.) a surface area between about 2.5 m²/g and about 6.0 m²/g; or
b) a surface area of about 3.0 m²/g or greater.

3. The fiber web of any one of claims 1-2, wherein the fiber web has a mean pore size between about 5 microns and about 15 microns.

4. The fiber web of any one of claims 1-3, wherein the fiber web has
a.) a basis weight between about 3.0 g/m² and about 30 g/m²; or
b.) a consistency of basis weight across the fiber web of about 3.0 standard deviations or less.

5. The fiber web of any one of claims 1-4, wherein the fiber web has
a.) a thickness between about 0.05 mm (0.002 inches) and about 0,25 mm (0.010 inches); or
b.) a consistency of thickness across the fiber web of about 3.0 standard deviations or less.

6. The fiber web of any one of claims 1-5, wherein the fiber web has
a.) an air permeability between about 1.1 m³/min (40 CFM) and about 21.2 m³/min (750 CFM); or
b.) an air permeability between about 0.28 m³/min (10 CFM) and about 1.4 m³/min (50 CFM); or
c.) an airflow resistance between about 0.3 mm H₂O and about 3.5 mm H₂O; or
d.) a NaCl filtration efficiency between about 50% and about 99.97%.

7. The fiber web of any one of claims 1-6, wherein the a plurality of meltblown fibers have
a.) an average fiber diameter between about 0.1 microns and about 1.0 microns; or
b.) an average fiber diameter of less than about 1.0 microns; or
c.) an average fiber diameter of less than about 0.6 microns.

8. The fiber web of any one of claims 1-7, wherein the fiber web has
a.) a surface density of particles formed of the polymeric material of less than about 0.775 particles/cm² (5.0 particles/in²), wherein each of the particles has a largest cross-sectional dimension of about 1.0 mm or greater; or
b.) a surface density of particles formed of the polymeric material of less than about 0.465 particles/cm² (3.0 particles/in²), wherein each of the particles has a largest cross-sectional dimension of about 1.0 mm or greater; or
c.) a surface density of particles formed of the polymeric material of less than about 0.310 particles/cm² (2.0 particles/in²), wherein each of the particles has a largest cross-sectional dimension of about 1.0 mm or greater; or
d.) a surface density of particles formed of the polymeric material of less than about 0.248 particles/cm² (1.6 particles/in²), wherein each of the particles has a largest cross-sectional dimension of about 1.0 mm or greater; or
e.) a surface density of particles formed of the polymeric material of less than about 0.155 particles/cm² (1.0 particles/in²), wherein each of the particles has a largest cross-sectional dimension of about 1.0 mm or greater; or
f.) a surface density of particles formed of the polymeric material of less than about 0.109 particles/cm² (0.7 particles/in²), wherein each of the particles has a largest cross-sectional dimension of about 1.0 mm or greater; or
g.) a surface density of particles formed of the polymeric material of less than about 0.0775 particles/cm² (0.5 particles/in²), wherein each of the particles has a largest cross-sectional dimension of about 1.0 mm or greater; or
h.) a surface density of particles formed of the polymeric material of less than about 0.0465 particles/cm² (0.3 particles/in²), wherein each of the particles has a largest cross-sectional dimension of about 1.0 mm or greater.

9. The fiber web of any one of claims 1-8, wherein the fiber web comprises a fatty acid amide additive.

10. A filter element comprising the fiber web of any one of claims 1-9.

11. The fiber web of any one of claims 1-9, wherein the plurality of fibers have a standard deviation of fiber diameter of greater than 0.40 microns.

## Patentansprüche

1. Fasergewebe, umfassend:
eine Mehrzahl von schmelzgeblasenen Fasern mit einem durchschnittlichen Faserdurchmesser zwischen etwa 0,1 µm und etwa 1,5 µm, wobei das Fasergewebe aufweist:
eine Luftpermeabilität, gemessen gemäß dem Standard ASTM D737-75, zwischen etwa 0,283 m³/min (10 CFM) und etwa 51,0 m³/min (1800 CFM);
eine Oberfläche, die größer ist als etwa 2,0 m²/g, wobei die Oberfläche gemessen wird unter Verwendung eines BET-Oberflächenanalyzers gemäß Section 10 von Battery Council International Standard BCIS-03A;
ein Basisgewicht, bestimmt gemäß ASTM D3776, zwischen etwa 1,0 g/m² und etwa 100 g/m²; und
eine Dicke, bestimmt gemäß dem Standard ASTM D1777, zwischen etwa 0,0127 mm (0,0005 Zoll) und etwa 1,016 mm (0,04 Zoll).

2. Fasergewebe gemäß Anspruch 1, wobei das Fasergewebe aufweist
a.) eine Oberfläche zwischen etwa 2,5 m²/g und etwa 6,0 m²/g; oder
b) eine Oberfläche von etwa 3,0 m²/g oder größer.

3. Fasergewebe gemäß einem der Ansprüche 1 bis 2, wobei das Fasergewebe eine mittlere Porengröße zwischen etwa 5 µm und etwa 15 µm aufweist.

4. Fasergewebe gemäß einem der Ansprüche 1 bis 3, wobei das Fasergewebe aufweist
a.) ein Basisgewicht zwischen etwa 3,0 g/m² und etwa 3,0 g/m²; oder
b.) eine Konsistenz des Basisgewichts über das Filtergewebe von etwa 3,0 Standardabweichungen oder weniger.

5. Fasergewebe gemäß einem der Ansprüche 1 bis 4, wobei das Fasergewebe aufweist
a.) eine Dicke zwischen etwa 0,05 mm (0,002 Zoll) und etwa 0,25 mm (0,010 Zoll); oder
b.) eine Konsistenz der Dicke über das Fasergewebe von etwa 3,0 Standardabweichungen oder weniger.

6. Fasergewebe gemäß einem der Ansprüche 1 bis 5, wobei das Fasergewebe aufweist
a.) eine Luftpermeabilität zwischen etwa 1,1 m³/min (40 CFM) und etwa 21,2 m³/min (750 CFM); oder
b.) eine Luftpermeabilität zwischen etwa 028 m³/min (10 CFM) und etwa 1,4 m³/min (50 CFM); oder
c.) einen Luftstromwiderstand zwischen etwa 0,3 mm H₂O und etwa 3,5 mm H₂O; oder
d.) eine NaCl-Filtrationseffizienz zwischen etwa 50 % und etwa 99,97 %.

7. Fasergewebe gemäß einem der Ansprüche 1 bis 6, wobei die Mehrzahl von schmelzgeblasenen Fasern aufweist
a.) einen durchschnittlichen Faserdurchmesser zwischen etwa 0,1 µm und etwa 1,0 µm, oder
b.) einen durchschnittlichen Faserdurchmesser von weniger als etwa 1,0 µm; oder
c.) einen durchschnittlichen Faserdurchmesser von weniger als etwa 0,6 µm.

8. Fasergewebe gemäß einem der Ansprüche 1 bis 7, wobei das Fasergewebe aufweist
a.) eine Oberflächendichte an aus dem Polymermaterial gebildeten Partikeln von weniger als etwa 0,775 Partikel/cm² (5,0 Partikel/Zoll²), wobei jedes der Partikeln eine größte Querschnittsdimension von etwa 1,0 mm oder größer aufweist; oder
b.) eine Oberflächendichte an aus dem Polymermaterial gebildeten Partikeln von weniger als etwa 0,465 Partikel/cm² (3,0 Partikel/Zoll²), wobei jedes der Partikeln eine größte Querschnittsdimension von etwa 1,0 mm oder größer aufweist; oder
c.) eine Oberflächendichte an aus dem Polymermaterial gebildeten Partikeln von weniger als etwa 0,310 Partikel/cm² (2,0 Partikel/Zoll²), wobei jedes der Partikeln eine größte Querschnittsdimension von etwa 1,0 mm oder größer aufweist; oder
d.) eine Oberflächendichte an aus dem Polymermaterial gebildeten Partikeln von weniger als etwa 0,248 Partikel/cm² (1,6 Partikel/Zoll²), wobei jedes der Partikeln eine größte Querschnittsdimension von etwa 1,0 mm oder größer aufweist; oder
e.) eine Oberflächendichte an aus dem Polymermaterial gebildeten Partikeln von weniger als etwa 0,155 Partikel/cm² (1,0 Partikel/Zoll²), wobei jedes der Partikeln eine größte Querschnittsdimension von etwa 1,0 mm oder größer aufweist; oder
f.) eine Oberflächendichte an aus dem Polymermaterial gebildeten Partikeln von weniger als etwa 0,109 Partikel/cm² (0,7 Partikel/Zoll²), wobei jedes der Partikeln eine größte Querschnittsdimension von etwa 1,0 mm oder größer aufweist; oder
g.) eine Oberflächendichte an aus dem Polymermaterial gebildeten Partikeln von weniger als etwa 0,0775 Partikel/cm² (0,5 Partikel/Zoll²), wobei jedes der Partikeln eine größte Querschnittsdimension von etwa 1,0 mm oder größer aufweist; oder
h.) eine Oberflächendichte an aus dem Polymermaterial gebildeten Partikeln von weniger als etwa 0,0465 Partikel/cm² (0,3 Partikel/Zoll²), wobei jedes der Partikeln eine größte Querschnittsdimension von etwa 1,0 mm oder größer aufweist; oder

9. Fasergewebe gemäß einem der Ansprüche 1 bis 8, wobei das Fasergewebe ein Fettsäureamidadditiv umfasst.

10. Filterelement, umfassend das Fasergewebe gemäß einem der Ansprüche 1 bis 9.

11. Fasergewebe gemäß einem der Ansprüche 1 bis 9, wobei die Mehrzahl von Fasern eine Standardabweichung des Faserdurchmessers von größer als 0,40 µm aufweist.

## Revendications

1. Voile de fibres comprenant:
une pluralité de fibres extrudées par soufflage ayant un diamètre de fibres moyen entre environ 0,1 micron et environ 1,5 micron, dans lequel le voile de fibres a :
- une perméabilité à l'air mesurée selon la norme ASTM D737-75 entre environ 0,283 m³/min (10 CFM) et environ 51,0 m³/min (1 800 CFM) ;
- une aire de surface supérieure à environ 2,0 m²/g, dans lequel l'aire de surface est mesurée en utilisant un analyseur de surface Brunauer-Emmett-Teller (BET) conformément à la section 10 de la norme BCIS-03A du Battery Council International ;
- un poids de base déterminé selon ASTM D3776 entre environ 1,0 g/m² et environ 100 g/m²; et
- une épaisseur déterminée selon la norme ASTM D1777 entre environ 0,0127 mm (0,0005 pouce) et environ 1,016 mm (0,04 pouce).

2. Voile de fibres selon la revendication 1, dans lequel le voile de fibres a
a.) une aire de surface entre environ 2,5 m²/g et environ 6,0 m²/g ; ou
b) une aire de surface supérieure ou égale à environ 3,0 m²/g.

3. Voile de fibres selon l'une quelconque des revendications 1 et 2, dans lequel le voile de fibres a une taille de pore moyenne entre environ 5 microns et environ 15 microns.

4. Voile de fibres selon l'une quelconque des revendications 1 à 3, dans lequel le voile de fibres a
a.) un poids de base entre environ 3,0 g/m² et environ 30 g/m²; ou
b.) une uniformité de poids de base sur le voile de fibres inférieure ou égale à environ 3,0 d'écart type.

5. Voile de fibres selon l'une quelconque des revendications 1 à 4, dans lequel le voile de fibres a
a.) une épaisseur entre environ 0,05 mm (0,002 pouce) et environ 0,25 mm (0,010 pouce) ; ou
b.) une uniformité d'épaisseur sur le voile de fibres inférieure ou égale à environ 3,0 d'écart type.

6. Voile de fibres selon l'une quelconque des revendications 1 à 5, dans lequel le voile de fibres a
a.) une perméabilité à l'air entre environ 1,1 m³/min (40 CFM) et environ 21,2 m³/min (750 CFM) ; ou
b.) une perméabilité à l'air entre environ 0,28 m³/min (10 CFM) et environ 1,4 m³/min (50 CFM) ; ou
c.) une résistance à l'écoulement d'air entre environ 0,3 mm de H₂O et environ 3,5 mm de H₂O; ou
d.) une efficacité de filtration de NaCl entre environ 50 % et environ 99,97 %.

7. Voile de fibres selon l'une quelconque des revendications 1 à 6, dans lequel la une pluralité de fibres extrudées par soufflage a
a.) un diamètre de fibre moyen entre environ 0,1 micron et environ 1,0 micron ; ou
b.) un diamètre de fibre moyen inférieur à environ 1,0 micron ; ou
c.) un diamètre de fibre moyen inférieur à environ 0,6 micron.

8. Voile de fibres selon l'une quelconque des revendications 1 à 7, dans lequel le voile de fibres a
a.) une densité de surface de particules formées du matériau polymère inférieure à environ 0,775 particule/cm² (5,0 particules/po²), dans lequel chacune des particules a une dimension transversale maximale supérieure ou égale à environ 1,0 mm ; ou
b.) une densité de surface de particules formées du matériau polymère inférieure à environ 0,465 particule/cm² (3,0 particules/po²), dans lequel chacune des particules a une dimension transversale maximale supérieure ou égale à environ 1,0 mm ; ou
c.) une densité de surface de particules formées du matériau polymère inférieure à environ 0,310 particule/cm² (2,0 particules/po²), dans lequel chacune des particules a une dimension transversale maximale supérieure ou égale à environ 1,0 mm ; ou
d.) une densité de surface de particules formées du matériau polymère inférieure à environ 0,248 particule/cm² (1,6 particule/po²), dans lequel chacune des particules a une dimension transversale maximale supérieure ou égale à environ 1,0 mm ; ou
e.) une densité de surface de particules formées du matériau polymère inférieure à environ 0,155 particule/cm² (1,0 particule/po²), dans lequel chacune des particules a une dimension transversale maximale supérieure ou égale à environ 1,0 mm ; ou
f.) une densité de surface de particules formées du matériau polymère inférieure à environ 0,109 particule/cm² (0,7 particule/po²), dans lequel chacune des particules a une dimension transversale maximale supérieure ou égale à environ 1,0 mm ; ou
g.) une densité de surface de particules formées du matériau polymère inférieure à environ 0,0775 particule/cm² (0,5 particule/po²), dans lequel chacune des particules a une dimension transversale maximale supérieure ou égale à environ 1,0 mm ; ou
h.) une densité de surface de particules formées du matériau polymère inférieure à environ 0,0465 particule/cm² (0,3 particule/po²), dans lequel chacune des particules a une dimension transversale maximale supérieure ou égale à environ 1,0 mm.

9. Voile de fibres selon l'une quelconque des revendications 1 à 8, dans lequel le voile de fibres comprend un additif d'amide d'acide gras.

10. Élément filtre comprenant le voile de fibres selon l'une quelconque des revendications 1 à 9.

11. Voile de fibres selon l'une quelconque des revendications 1 à 9, dans lequel la pluralité de fibres a un écart type de diamètre de fibre supérieur à 0,40 micron.
